

# United States Patent Office.

R. SANDS TUCKER, OF BROOKLYN, NEW YORK.

*Letters Patent No. 62,236, dated February 19, 1867.*

## IMPROVED COMPOUND FOR COATING AND INSULATING TELEGRAPHIC WIRES.

The Schedule referred to in these Letters Patent and making part of the same.

### TO ALL WHOM IT MAY CONCERN:

Be it known that I, RICHARD SANDS TUCKER, of the city of Brooklyn, county of Kings, and State of New York, have invented a new and improved Method of Manufacturing a Covering or Insulator for Metallic Wires or Conductors used in submarine or other telegraphing, and also an improved mode of manufacturing a paint, varnish, or covering, to be used in the protection of structures of all kinds. Specimens of the said insulator, of said paint or covering, and of the materials composing the same, accompany this application.

The nature of my invention consists in combining glass finely ground or pulverized with linseed oil or other oleaginous or resinous substances; and for the purpose of insulating telegraph wires I saturate yarns of hemp with a compound composed of the said glass combined with the said linseed oil, tar, or other oleaginous or resinous substances, and closely surround and circumvolute the conducting wire or wires with said yarns. I then surround the said insulator with a covering of wire or tarred hempen yarn, or both, as an armor to protect it from external injury and to strengthen the same.

For the manufacture of said paint, varnish, or covering, I incorporate by mixing the said pulverized glass with linseed oil or other oleaginous substance.

What I claim as my invention, and desire to secure by Letters Patent, is—

My application of glass finely ground or pulverized, and mixed or incorporated with linseed oil, tar, or other oleaginous and resinous substances, to insulate metallic wires or conductors in telegraph cables.

R. SANDS TUCKER.

Witnesses:

EPHM. R. SALE,

J. A. TUCKER.